

## UNITED STATES PATENT OFFICE

2,403,284

PHOSPHATIDIC LUBRICANT AND METHOD  
OF MAKINGJoseph J. Jacobs, Brooklyn, N. Y., assignor to  
American Lecithin Company, Cleveland, Ohio,  
a corporation of OhioNo Drawing. Application September 3, 1943,  
Serial No. 501,173

7 Claims. (CL. 252—51)

1

This invention relates generally to the art of phosphatides and more particularly to a new and improved phosphatide composition of special value as an additive to mineral lubricating oils and greases, to a new and improved method of making such composition, and to new and improved mineral lubricating oils and greases.

Mineral lubricating oils tend to deteriorate or decompose under certain severe operating conditions to which they are often subjected in use, for example, in internal combustion engines, electric motors, high pressure bearings and the like. In use, these oils and greases may deteriorate by being oxidized with the resultant formation of corrosive acids which corrode certain metals and alloys, particularly bearing metal containing cadmium-silver or copper-lead alloys, and such corrosion may be of critical importance where high strength alloys are required to carry heavy loads. These oils also deteriorate or decompose by being cracked, or oxidized, and then polymerized with resultant increase of viscosity or formation of resinous compounds, or both. Excessive wear of engine parts, loss of engine power and the sticking or freezing of metal parts, such as rings in piston ring grooves, and increased costs of engine operation and maintenance may result from these increases in viscosity or formations of resinous compounds.

Various efforts have been made heretofore to increase the resistance of lubricating oils and greases to deterioration or decomposition when subjected to severe operating conditions. These efforts have included the use of additives, that is, compounds which were added to the oils and greases and which consisted of phenols, halogenated materials, phosphorous compounds, certain amines, metallic compounds and commercial soybean lecithin. However, so far as I know, none of these additives has been entirely satisfactory.

The present invention is predicated on the discovery that compounds made by suitable treatment of vegetable phosphatides are quite valuable as lubricants and as additives to lubricants. The compounds embodying the present invention may be used alone as lubricants for gears and bearings which are subjected to high pressures or may be added to mineral lubricating oils which are subjected to high temperatures, or mixed with greases which are to be used on metal-bearing surfaces subjected to high temperatures or high pressures.

Briefly stated, compositions embodying the present invention may be made by blending vegetable phosphatides with petroleum hydrocarbon

5 oils in varying proportions and subjecting the blend to elevated temperatures. While I prefer to prepare the compounds of this invention by heating a mixture of a vegetable phosphatide and mineral lubricating oil in the presence of a catalyst and while passing air thru the mixture, compounds comparable in results to those so produced may be made by omitting the catalysts or air or both.

10 This invention will be better understood by those skilled in the art from the following examples of the compositions and process which are set forth by way of illustration but not of limitation.

## Example I

15 100 parts of commercial soybean phosphatide were dissolved in 100 parts of an SAE 30 Mid-Continent petroleum distillate of lubricating oil grade and the resulting solution or mixture was heated for 24 hours at 325° F. in the presence of catalysts comprising strips of low carbon steel and copper and while air was bubbling thru the liquid at the rate of 30 liters per hour. During 20 the treatment foaming occurred and the liquid took on a darker color. Compositions with comparable properties were obtained by similarly heating other quantities of the foregoing composition in the presence of the catalysts but without air bubbling thru, with bubbling air and no catalyst and with neither bubbling air nor catalyst.

## Example II

25 35 Equal parts of a commercial lecithin product containing a carrier of 30% soybean oil and a mineral lubricating oil were heated for one hour at 325° F. in the presence of a low carbon steel catalyst in bulk form. Compositions with comparable properties were obtained by heating other quantities of the foregoing composition without the catalyst, with the catalyst and air bubbling thru at the rate of 30 liters per hour, and with the air but without the catalyst.

40 45 The new, unexpected and unpredictable properties possessed by compounds of the foregoing examples when used as additives to lubricating oils are shown by the following illustrations:

Illustration A.—1% of the compound produced 50 in accordance with Example I was added to a solvent-refined mineral lubricating oil of motor oil viscosity range and that mixture was tested against a quantity of the same oil containing no additive and another quantity of the same oil containing .5% of commercial soybean lecithin.

At the end of 70 hours of accelerated testing the following comparative results were obtained:

|                                          | No.<br>additive | 0.5% com-<br>mercial<br>soybean<br>lecithin | 1% com-<br>position<br>Example<br>No. 1 |
|------------------------------------------|-----------------|---------------------------------------------|-----------------------------------------|
| Percent increase in viscosity at 100° F. | 100             | 33.6                                        | 1.25                                    |
| Naphtha insoluble mgs./10 gms. oil       | 307             | 135                                         | 146                                     |
| Neutralization number                    | 3.1             | 0.9                                         | 0.3                                     |

These results indicate that the lubricating oil to which the composition of Example I was added was improved to a surprising extent as compared with the other oils. The extremely small percentage increase in viscosity is important because it indicates that the oil did not polymerize to any noticeable extent during the test while the neutralization number indicates that the oil oxidized to a very small extent and, therefore, formed but little acid. The small difference in naphtha-insoluble material between the two oils containing the additives is insignificant as compared with the large amount of that material in the additive-free oil. That material results from oxidation. These results indicate the new and unexpected superior inhibiting properties of a composition of this invention.

*Illustration B.*—A quantity of the compound resulting from the treatment outlined in Example I hereinabove was filtered to separate out the insoluble material and the filtrate was added to an SAE 30 conventionally refined Pennsylvania motor oil to the extent of 1% thereof. This oil was compared with a quantity of the same motor oil to which was added .5% of soybean phosphatides. These two oils were subjected to the same test for a period of 64 hours with the following results:

|                                       | 0.5% soybean<br>phosphatides | 1% composition<br>No. 1<br>filtered |
|---------------------------------------|------------------------------|-------------------------------------|
| Viscosity increase at 100° F. percent | 54.4                         | 27.8                                |
| 210° F. do                            | 27.8                         | 12.1                                |
| Naphtha insolubles, mgs./10 gms. oil  | 60.0                         | 4.2                                 |
| Neutralization number                 | 3.8                          | 1.67                                |
| Varnish rating                        | 4                            | 2                                   |

It will be noted that the inhibiting properties of the filtered composition embodying the present invention were far superior to those of the ordinary soybean phosphatides in all respects including varnish rating which is an index of the tendency of the oil to deteriorate or decompose with the formation of lacquer or varnish on engine parts. The varnish rating range is from 0 to 10.

The results set out in illustrations A and B are representative of results obtainable with the compounds of Examples I and II with mineral lubricating oils of motor oil viscosity range from different localities and whether solvent-refined or conventionally refined.

It is to be understood that Examples I and II do not show the full range of oil and phosphatide or lecithin percentages which may be used in preparing the new compositions. In general, the oil content in the mixture to be treated by the present process may range from about 10% to about 90% of phosphatide or lecithin.

While illustrations A and B show the results of using oils containing 1% of the compounds embodying this invention, it is to be understood

that such percentage may be varied from about .02% to about 15%, the higher portion of that percentage range, that is, from about 5% to about 15% being particularly applicable to greases.

The length of time of heating of the mixture of oil and phosphatides may vary considerably, as is indicated by Examples I and II where the times were 24 hours and one hour respectively.

Altho the temperatures shown in Examples I and II are the same, 325° F., other temperature ranging between about 200° F. and about 375° F. may be used with comparable results. In general, heating at a lower temperature for a longer time will accomplish results similar to heating at a higher temperature for a shorter time.

Compounds embodying the present invention may be used alone as lubricants under certain conditions, for example, on glass or on high pressure bearings.

Having thus described the invention so that others skilled in the art may be able to understand and practice the same, I state that what I desire to secure by Letters Patent is defined in what is claimed.

What is claimed is:

1. A new composition having the properties of inhibiting the oxidation of, and the formation of naphtha insolubles in, a mineral lubricating oil and consisting of a vegetable phosphatide and from 10% to 90% of a mineral oil, said mixture having been heated at a temperature of between about 200° F. and 375° F. for between one hour and twenty-four hours in the presence of an oxidation promoting catalyst while air was passed thru the mixture at the rate of about 30 liters per hour.

2. A new composition having the properties of inhibiting the oxidation of, and the formation of naphtha insolubles in, a mineral lubricating oil and consisting of a vegetable phosphatide and from 10% to 90% of a mineral oil, said mixture having been heated at a temperature of between about 200° F. and 375° F. for between one hour and twenty-four hours.

3. A new composition having the properties of inhibiting the oxidation of, and the formation of naphtha insolubles in, a mineral lubricating oil and consisting of a vegetable phosphatide and from 10% to 90% of a mineral oil, said mixture having been heated at a temperature between about 200° F. and about 375° F. for between 1 hour and 24 hours in the presence of an oxidation promoting catalyst.

4. A new composition having the properties of inhibiting the oxidation of, and the formation of naphtha insolubles in, a mineral lubricating oil and consisting of a vegetable phosphatide and from 10% to 90% of a mineral oil, said mixture having been heated at a temperature between about 200° F. and about 375° F. for between 1 hour and 24 hours while air was passed thru the mixture.

5. A lubricant comprising a mineral lubricating oil containing between about .02% and about 15% of a composition having the properties of inhibiting the oxidation of, and the formation of naphtha insolubles in, said oil and consisting of a vegetable phosphatide and from 10% to 90% of a mineral oil, said mixture having been heated at a temperature of from about 200° F. to about 375° F. for between 1 hour and 24 hours before being added to said lubricating oil.

6. A lubricant in the form of a mineral lubricating oil containing between about .02% and

5% of a composition having the properties of inhibiting the oxidation of, and the formation of naphtha insolubles in, said lubricating oil and consisting of a vegetable phosphatide and from 10% to 90% of a mineral oil, said mixture having been heated at a temperature of from about 200° F. to about 375° F. for between 1 hour and 24 hours prior to addition of the mixture to said lubricating oil.

7. A lubricant in the form of a mineral lubri- 10

cating grease containing between about 5% and 15% of a composition having the properties of inhibiting the oxidation of, and the formation of naphtha insolubles in, said grease and consisting of a vegetable phosphatide and from 10% to 90% of a mineral oil, said mixture having been heated at a temperature of from about 200° F. to about 375° F. for between 1 hour and 24 hours before being added to said grease.

JOSEPH J. JACOBS.